

## UNITED STATES PATENT OFFICE

PHILIP S. DANNER, OF POINT RICHMOND, CALIFORNIA, ASSIGNOR TO STANDARD OIL COMPANY OF CALIFORNIA, OF SAN FRANCISCO, CALIFORNIA, A CORPORATION OF DELAWARE

## NONDETONATING FUEL

No Drawing. Original application filed June 19, 1926, Serial No. 117,153. Divided and this application filed March 1, 1928, Serial No. 258,440. Renewed December 21, 1931.

This invention relates to a motor fuel, and particularly refers to a motor fuel of the so-called non-detonating type. This application is a division of my co-pending application Serial No. 117,153 filed June 19, 1926.

The hydrocarbon motor fuels now in use all have a very definite break down or detonation point beyond which the fuels cannot be used without serious trouble arising in the operation of the internal combustion engine. When the compression pressure is raised, a definite or critical pressure is reached at which each particular motor fuel produces a decided knock. This knocking is evidenced by a pinking sound in the motor combustion chamber and is accompanied by a loss in power, overheating, and eventual pre-ignition which, if severe, will cause the motor to stop.

One of the principal objects of the present invention is to provide a motor fuel for use in internal combustion engines which possesses less detonating properties than motor fuel now in use. It has been found that certain relatively unstable organic compounds of metals, when admixed with mineral motor fuel, operate to suppress detonation in internal combustion engines operating under relatively large loads and that high compression ratios, for example compression ratios in excess of about 4.5 to 1, may be employed when using such materials. Among the organic compounds of metal which have been employed for suppressing detonation in internal combustion engines is iron carbonyl

35  $\text{Fe}(\text{CO})_5$ , a material more properly known as iron pentacarbonyl. This material operates very satisfactorily in suppressing detonation in internal combustion engines but has the disadvantage that it is unstable in the presence of air, light and moisture and difficulty is experienced in using motor fuels containing the iron pentacarbonyl due to the rapidity with which the pentacarbonyl decomposes upon standing. I have discovered that the tetracarbonyl of iron  $\text{Fe}(\text{CO})_4$  is not only an efficient agent for suppressing detonation in an internal combustion engine but that when added to motor fuel it is highly stable on exposure to air, moisture and light.

50 Therefore the present invention involves dis-

covery of a non-detonating fuel of exceptional stability with respect to air, light and moisture.

Various further objects, advantages and features of the present invention will be apparent from the description of a preferred form or forms of non-detonating fuel embodying the invention.

The base of the motor fuel comprises a mineral hydrocarbon oil of any desired type such as is usually obtained from petroleum oil. To this mineral motor fuel is added quantities of iron tetracarbonyl which may considerably vary, depending upon the compression ratio of the internal combustion engine in which the motor fuel is to be employed. As an example of such motor fuel, iron tetracarbonyl has been added to gasoline from California crude petroleum oil in proportions of approximately 5 to 10 grams of carbonyl per gallon of gasoline. The fuel thus prepared, when used to operate a motor with a compression ratio of as high as from 5.4 to 6.0 to 1, will operate satisfactorily without detonation. Obviously the greater the ratio of the carbonyl to the gasoline the higher the compression ratio of the engine may be.

While I have described the preferred form or forms of motor fuel embodying the present invention, it is understood that the invention is not limited to the specific form described but is of the scope set forth in the accompanying claims.

I claim:

1. A non-detonating motor fuel comprising a mineral hydrocarbon oil admixed with iron tetracarbonyl.

2. A non-detonating motor fuel comprising, an admixture of mineral hydrocarbon oil in iron tetracarbonyl in sufficient proportion to permit the fuel to operate without self-detonation under compression ratios above 5.4 to 1.

3. A non-detonating motor fuel comprising a hydrocarbon motor fuel in combination with between about .1 and 1 percent of iron tetracarbonyl.

Signed at Point Richmond, Cal., this 9th day of February, 1928.

PHILIP S. DANNER. 100